

# UNITED STATES PATENT OFFICE.

PAUL BENRATH, OF MULHEIM, NEAR COLOGNE, AND ERNST DAMM AND OTTO STEPHANI, OF ELBERFELD, GERMANY, ASSIGNEES TO FARBENFABRIKEN VORM. FRIEDR. BAYER & CO., OF ELBERFELD, GERMANY, A CORPORATION OF GERMANY.

## LUSTROUS THREAD.

1,031,616.

Specification of Letters Patent. Patented July 2, 1912.

No Drawing.

Application filed October 28, 1909. Serial No. 525,175.

*To all whom it may concern:*

Be it known that we, PAUL BENRATH, residing at Mulheim, near Cologne, and ERNST DAMM and OTTO STEPHANI, residing at Elberfeld, in the Kingdom of Prussia, Germany, citizens of the German Empire, have invented new and useful Improvements 5 in Lustrous Threads, of which the following is a specification.

10 To produce threads, bands, etc., having a metallic luster, it has been necessary heretofore to wrap threads of metal around textile threads. The chief drawback to this process is the difficulty of producing a firm adhesion 15 of the metal to the thread, and lustrous threads prepared in this manner are not very durable. We have now found that, according to the process hereinafter described, threads having a metallic luster can be obtained 20 in which the metal producing the luster adheres firmly to the threads.

To produce our new lustrous threads, threads spun from cotton, flax, wool, silk, 25 gum or metallic threads, wires or bands are passed through a mixture of metallic bronzes or powders with solutions of cellulose acetates with or without the addition of other suitable pigments to insure a homogeneous mixture of the bronzes with the 30 solutions. The threads on emerging from this mixture are then finished by polishing, pressing, filing, etc.

Example 1: A cotton thread is drawn slowly through chloroform containing in solution 35 5 per cent. of acetylated cellulose (see United States Letters Patent 790565) and in suspension 15 per cent. of goldbronze. The thread on emerging from the chloroform is wound up.

40 Example 2: A cotton thread is drawn through a solution of acetylated cellulose and is then drawn slowly through acetone containing in solution 10 per cent. of acetylated cellulose (see British Letters Patent 45 24067 of 1906) and in suspension 30 per cent. of copper bronze. The thread on emerging from the acetone is then drawn through a third solution of acetylated cellulose and wound up.

50 This new material splits off acetic acid if it is digested for several days with dilute sulfuric acid. On distillation with steam,

acetic acid distils over and the quantity of it may be ascertained by titration or by any other known method.

On using dyed bronzes or a solution of the acetylated cellulose containing a dye various shades can be obtained.

Where threads or bands are thus treated, the adhesion of the acetylcellulose thereto is 60 greatly enhanced by the presence of the metal powder in the ester coating. This is due in part to the fact that the rate of expansion and contraction of the coating as a whole is brought nearer that of the core; 65 and this is especially true where the core is a metal thread. With cores of cotton, silk, or wool fibers and the like, there is more or less impregnation as well as coating of the core by the acetylcellulose solution, and consequently upon evaporation of the solvent 70 the layer of set acetylcellulose is firmly locked to the core. On the other hand, the metal powder, and the other pigments if present, do not penetrate the core to any 75 extent, remaining largely as a superficial layer of discrete metallic particles or flakes, each incased by and incorporated with the set but elastic and flexible acetylcellulose. The coating may appear continuous, but 80 there is substantially no actual contact between the metallic particles by reason of the intervening ester film linking adjacent particles. As a result, the metallic finish coating of threads made in this way, whether 85 with metallic or non-metallic cores, is consequently exceedingly flexible as well as adherent.

For the purposes of the present invention, the core of the new lustrous thread may be 90 of any permeable material capable of being impregnated with the acetyl cellulose solution to an extent sufficient to give the type of locking union between core and coating herein contemplated.

We claim:

1. As a new article of manufacture, a lustrous thread comprising a core of permeable material provided with a coating of acetylcellulose in which is incorporated a metal 100 powder, said coating being firmly locked to said core.

2. As a new article of manufacture, a lustrous thread comprising a thread of fibrous

material provided with a coating of acetyl-cellulose in which is incorporated a metal powder, said coating being firmly locked to said thread.

5. As a new article of manufacture, a lustrous thread comprising a core of cotton impregnated and coated with acetylcellulose carrying an incorporated metal powder.

10. As a new article of manufacture, a lustrous thread comprising a core of fibrous material provided with a coating of acetyl-cellulose firmly locked thereto, said coating

containing incorporated metal powder and coloring matter.

In testimony whereof we have hereunto 15 set our hands in the presence of two subscribing witnesses.

PAUL BENRATH. [L.S.]  
ERNST DAMM. [L.S.]  
OTTO STEPHANI. [L.S.]

Witnesses:

OTTO KÖNIG,  
CHAS. J. WRIGHT.